

## UNITED STATES PATENT OFFICE

ALAN KIESOCK, OF FOREST HILLS, NEW YORK

## MOLYBDENUM ALLOY IRON AND STEEL

No Drawing.

Application filed November 15, 1927. Serial No. 233,521.

The invention relates to a new and useful material for producing molybdenum alloys of iron and steel, and more particularly to a novel and useful low-percentage, molybdenum-bearing pig iron suitable for use as such an alloying agent or material.

The main objects and advantages of my invention will be set forth in part hereinafter, and in part will be obvious herefrom, or may 10 be learned by practice with the invention.

Among the principal advantages of the molybdenum-bearing pig iron of my invention are its relatively low temperature melting point, whereby it lends itself most flexibly to the manufacture of alloy irons and steels in different ways and according to different processes, some of which will be described hereinafter. The percentages of molybdenum in my pig iron may be widely 15 varied so far as concerns the broader features of my invention, but these percentages will be kept within limits so that the iron will be fusible at usual steel and iron furnace temperatures. Another advantage of said product 20 of my invention is that it contains no molybdenum, and probably no other carbon compounds which are not dissociable at ordinary steel or iron furnace temperatures. Another advantage of this product of my invention 25 is that it does not require further reduction, but only intermixture, or melting together to effect the desired percentage alloy of the iron and steel, which intermixture may be effected at the ordinary and necessary 30 temperatures of the various iron or steel making operations, even such operations wherein relatively low temperatures prevail.

So far as concerns my present invention, it is broadly immaterial as to the manner in 40 which it is produced; however, the preferred process for producing the molybdenum pig iron of my invention is described and claimed in my copending application Ser. No. 230,381, filed November 1, 1927.

As set forth in said application, a molybdenum-containing compound or other suitable molybdenum-containing substance or material is added to the successive charges of a blast furnace, during the usual operation 45 thereof, the addition of such molybdenum

compound or other molybdenum-containing substance being in such quantity as to produce the desired percentage of molybdenum alloy in the pig iron which is the product of the furnace.

55

Various molybdenum compounds may be employed in producing the molybdenum-bearing pig iron of my process, as may be found convenient or desirable, such as molybdenum oxide, calcium molybdate, or molybdenum sulfide. If desired, there may be added to an ordinary blast furnace charge sufficient of the molybdenum compound of known metallic content to secure the desired or predetermined percentage of molybdenum 60 in the pig iron, as for example, to introduce four pounds of molybdenum for every one hundred pounds of iron contained in the charge. In view of the continuous operation and periodic charging of the blast furnace 65 with predetermined quantities of the charging materials, the molybdenum-bearing compound, in predetermined amount, may be included with any one of the charging materials. The percentage of molybdenum obtained in 70 the pig iron will be found practically equivalent to the predetermined percentage introduced into the furnace charge.

75

The molybdenum-containing compound introduced into the blast furnace charge in the 80 manner described, or any other suitable manner during the operation goes down through the furnace with the other ingredients of the charge and is progressively subjected to the smelting or reducing operation of the furnace. 85 As the furnace operation proceeds and the charge materials are subjected to the gradually increasing temperatures and progress to a state of complete fusibility, the molybdenum is released from its compound and is absorbed practically completely into the liquid iron as a permanent alloy thereof in the predetermined percentage proportion.

90

I do not wish to be bound by any definite theory of the alloying process which proceeds 95 concurrently with the blast furnace operation, but it would appear that due to the relatively low affinity of molybdenum for oxygen and possibly due to the presence of powerful reducing agents, and the gradual and pro- 100

gressive temperature increase downwardly through the furnace, the molybdenum either directly or indirectly is completely reduced to the metallic state, and absorption thereof by the iron is insured, even at the temperatures prevailing in the blast furnace. In any event, substantially the entire molybdenum content of the molybdenum-bearing compound introduced into the charge will be transmitted as an alloy into the pig iron.

The product of my invention, molybdenum-bearing pig iron, provides a material for making a molybdenum alloy steel by the so called "hot-metal" process. In connection with this process, molten pig iron containing a known percentage of molybdenum may be taken from a blast furnace and added while still molten, in predetermined quantities, to the charge of the steel-making furnace. If more convenient or desirable, however, the solid molybdenum-bearing pig iron, in quantities sufficient to provide the percentage of molybdenum desired in the finished alloy steel, may be added to the original charge of the steel-making furnace.

Molybdenum-bearing pig iron is of particular advantage in the production of molybdenum grey, white, malleable or semi-steel castings as produced from metal melted in the ordinary cupola furnace.

It is impracticable to produce a molybdenum alloy from cupola iron with ferro-molybdenum by reason of its relatively high temperature melting point, the possible presence of undissociable carbides, together with lack of means for proper mixing, with consequent poor distribution of the molybdenum throughout the iron. The use of a molybdenum compound as an addition to the cupola ladle is unsatisfactory for the reason that at the prevailing temperatures sufficient time is not available for completion of the reducing reaction before the metal is too cool for casting, and efficient and complete mixing is impracticable.

The molybdenum pig iron of my invention likewise provides a most excellent and suitable material for addition to the charge of the cupola furnace to produce a desired molybdenum alloy for casting. It may be introduced as a part of the original charge of the cupola furnace in such relative proportion as to effect the desired percentage alloy of molybdenum in the product from the cupola furnace. It insures uniform distribution of the alloy throughout the product and without the introduction of any harmful impurities, whereby castings made from such alloy iron are of very superior quality and purity. Should it be desired, the molybdenum pig iron may be melted in a separate furnace, and the molten molybdenum-bearing pig iron therefrom be added in desired proportion to the output of a cupola which is melting ordinary iron.

What I claim is:—

1. An alloy to be used for alloying molybdenum with steel or iron comprising a molybdenum-bearing pig iron, the molybdenum content thereof being less than fifty per cent.

2. An alloy to be used for alloying molybdenum with steel or iron comprising a molybdenum-bearing pig iron, the molybdenum content thereof being approximately four per cent.

3. An alloy to be used for alloying molybdenum with steel or iron comprising a molybdenum-bearing pig iron, the molybdenum content thereof being approximately four per cent, and said pig iron being fusible at ordinary iron furnace temperatures.

In testimony whereof, I have signed my name to this specification.

ALAN KISSOCK.

70

75

80

85

90

95

100

105

110

115

120

125

130